

1

3,183,188

## PETROLEUM LUBRICANTS STABILIZED WITH BACTERICIDES

Edward B. Hodge, Terre Haute, Ind., assignor to Commercial Solvents Corporation, New York, N.Y., a corporation of Maryland  
No Drawing. Filed Mar. 20, 1961, Ser. No. 96,670  
11 Claims. (Cl. 252—49.5)

My invention relates to a stabilized petroleum lubricant and more particularly to a process for the production of stabilized petroleum lubricants containing as the active stabilizing agent nitrohexahydropyrimidines having the structural formula:



where R is lower alkyl and where R<sup>1</sup> is selected from the group consisting of lower alkyl and lower hydroxylalkyl.

It is well known that organisms from the groups consisting of *Corynebacterium*, *Achromobacter*, *Pseudomonas*, *Nocardia* and *Mycobacterium* metabolize petroleum hydrocarbons and fatty acids and thereby produce undesirable oxidation products.

The petroleum industry has long been interested in the stabilization of various petroleum products such as cutting oils, hydraulic fluids, etc., against breakdown by bacteria which metabolize the hydrocarbons with the concurrent formation of deleterious metabolites.

Many compounds have been used as stabilization agents in lubricants, but very few have been found to be commercially successful due to the fact that the compounds are unstable, or are not active against a wide variety of microorganisms.

Among the nitrohexahydropyrimidines having the above structural formula are included 1,3-bis(1-hydroxymethylpropyl)-5-methyl-5-nitrohexahydropyrimidine, 1,3-bis(2-hydroxyethyl)-5-methyl-5-nitrohexahydropyrimidine, 1,3,5-trimethyl-5-nitrohexahydropyrimidine, 5-ethyl-1,3-dimethyl-5-nitrohexahydropyrimidine, 5-ethyl-1,3-bis(2-ethylhexyl)-5-nitrohexahydropyrimidine, 1,3-dicyclohexyl-5-ethyl-5-nitrohexahydropyrimidine, 5-ethyl-1,3-bis(hydroxy-t-butyl)-5-nitrohexahydropyrimidine, and 5-ethyl-1,3-bis(2-hydroxypentyl)-5-nitrohexahydropyrimidine. I have found that in some instances I can obtain total inhibition of bacterial growth in petroleum lubricants at concentrations as low as 100 p.p.m. I prefer to include at least 1,000 p.p.m. in most petroleum formulations. However, I can employ amounts up to about 2% by weight of the active nitroamines when the latter is soluble to this extent in the particular petroleum hydrocarbon composition.

I have found that my active ingredients are effective bacteriostatic agents in petroleum containing lubricants such as cutting oils, penetrating oils, grinding lubricants, iron tinning lubricants, core oils, hydraulic fluids, etc.

The following examples set out lubricating compositions in which my active ingredients act as effective bacteriostatic agents. It is not intended that my invention be limited to the compositions, portions, or lubricants set out below; but rather I intend for all equivalents and variations obvious to those skilled in the art to be included within the scope of this specification and the attached claims.

### EXAMPLE I

To test the use of my active ingredients in cutting oils, a 25:1 water-cutting oil emulsion was prepared. The cut-

2

ting oil concentrate used was a proprietary cutting oil containing no bacterial inhibitors sold by Texaco Incorporated under the name of Soluble Oil Texaco-C. To each of one-gallon containers was added 1 liter of water-cutting oil emulsion. Desired amounts of my nitroamines were added to the cutting-oil emulsion in the first container. No inhibitor was added to the other container which was used as a control. At the beginning of the experiment, each unit was inoculated with 5 mls. of a heterogeneous bacterial culture which had grown for several years in a water-cutting oil emulsion. Aeration and mixing were obtained by using an air lift to continually circulate the mixture. The test was continued for a period of six weeks and during the six-week period, 5 mls. of bacterial culture were added at periodic weekly intervals.

The following table sets out the results of the above tests and the number of days of bacterial inhibition when the described concentration of the desired nitrohexahydropyrimidines were incorporated into the cutting-oil emulsion.

Table I

|    | Nitrohexahydropyrimidine                                           | Concentration<br>in 25:1<br>Water-Cutting<br>Oil Emulsion | Number<br>of Days<br>Effective |
|----|--------------------------------------------------------------------|-----------------------------------------------------------|--------------------------------|
| 25 | 1,3-bis(1-hydroxymethylpropyl)-5-methyl-5-nitrohexahydropyrimidine | 1,000                                                     | 14                             |
| 30 | 5-ethyl-1,3-bis(hydroxy-t-butyl)-5-nitrohexahydropyrimidine        | 1,000                                                     | >42                            |
|    | 5-ethyl-1,3-bis(hydroxy-t-butyl)-5-nitrohexahydropyrimidine        | 1,000                                                     | >42                            |
|    | Control                                                            |                                                           | 0                              |

### EXAMPLE II

The following is a water emulsifiable cutting oil which is adequately protected by 1,000 p.p.m. of my nitrohexahydropyrimidine inhibitors:

|    | Percent by weight    |
|----|----------------------|
| 40 | Light mineral oil 90 |
|    | Oleic acid 10        |

### EXAMPLE III

The following is a stabilized steam cylinder oil which is adequately protected by 1,000 p.p.m. of 5-ethyl-1,3-dimethyl-5-nitrohexahydropyrimidine.

|    | Percent                   |
|----|---------------------------|
| 45 | S.A.E. lubricating oil 90 |
|    | Oleic acid 10             |

### EXAMPLE IV

The following is a core oil which is adequately protected by 1,000 p.p.m. of 1,3,5-trimethyl-5-nitrohexahydropyrimidine.

|    | Percent                                |
|----|----------------------------------------|
| 55 | Crude tall oil 25                      |
|    | Fuel oil 35                            |
|    | Tall oil ester (glycol or glycerol) 40 |

### EXAMPLE V

The following is a cutting oil which is adequately protected by 1,000 p.p.m. of 1,3-bis(1-hydroxymethylpropyl)-5-methyl-5-nitrohexahydropyrimidine.

|    | Percent               |
|----|-----------------------|
| 65 | Tallow 65             |
|    | Paraffin wax 29       |
|    | Beeswax 1.3           |
| 70 | Oxalic acid 1.3       |
|    | Potassium citrate 1.3 |
|    | Urea 0.4              |

Now having described my invention, what I claim is:

1. A liquid petroleum composition consisting essentially of a liquid petroleum lubricant hydrocarbon and a sufficient amount of 1,3-bis(1-hydroxymethylpropyl)-5-methyl-5-nitrohexahydropyrimidine to stabilize said hydrocarbon against metabolizing bacteria.

2. A liquid petroleum composition consisting essentially of a liquid petroleum lubricant hydrocarbon and a sufficient amount of 1,3,5-trimethyl-5-nitrohexahydropyrimidine to stabilize said hydrocarbon against metabolizing bacteria.

3. A liquid petroleum composition consisting essentially of a liquid petroleum lubricant hydrocarbon and a sufficient amount of 5-ethyl-1,3-dimethyl-5-nitrohexahydropyrimidine to stabilize said hydrocarbon against metabolizing bacteria.

4. A liquid petroleum composition consisting essentially of a liquid petroleum lubricant hydrocarbon and a sufficient amount of 5-ethyl-1,3-bis(hydroxy-*t*-butyl)-5-nitrohexahydropyrimidine to stabilize said hydrocarbon against metabolizing bacteria.

5. An aqueous petroleum emulsion consisting essentially of an aqueous petroleum lubricant hydrocarbon emulsion and a sufficient amount of a nitrohexahydropyrimidine to stabilize said hydrocarbon against metabolizing bacteria, said nitrohexahydropyrimidine having the structural formula:



wherein R is lower alkyl and wherein R<sup>1</sup> is selected from the group consisting of lower alkyl and lower hydroxyalkyl.

6. A liquid petroleum composition consisting essentially of a liquid petroleum lubricant hydrocarbon and a sufficient amount of a nitrohexahydropyrimidine to stabilize said hydrocarbon against metabolizing bacteria,

5 said nitrohexahydropyrimidine having the structural formula:



10 wherein R is lower alkyl and wherein R<sup>1</sup> is selected from the group consisting of lower hydroxyalkyl and lower alkyl.

15 7. The composition of claim 6 wherein the composition is a cutting oil.

8. The composition of claim 6 wherein the composition is a steam cylinder oil.

20 9. The composition of claim 6 wherein the composition is a core oil.

10. The composition of claim 6 wherein the composition contains from about 100 p.p.m. to 2% by weight of the nitrohexahydropyrimidine.

25 11. The composition of claim 5 wherein the composition contains from about 100 p.p.m. to 2% by weight of the nitrohexahydropyrimidine.

#### References Cited by the Examiner

##### UNITED STATES PATENTS

|    |           |       |         |       |          |
|----|-----------|-------|---------|-------|----------|
| 80 | 2,391,847 | 12/45 | Senkus  | ----- | 260-251  |
|    | 2,812,332 | 11/57 | Pennino | ----- | 167-33   |
|    | 2,913,414 | 11/59 | Hodge   | ----- | 252-51.5 |
|    | 3,087,891 | 4/63  | Hodge   | ----- | 252-8.55 |

##### FOREIGN PATENTS

|         |      |            |
|---------|------|------------|
| 107,419 | 5/39 | Australia. |
| 160,367 | 1/55 | Australia. |
| 421,189 | 3/47 | Italy.     |

40 DANIEL E. WYMAN, Primary Examiner.

JULIUS GREENWALD, Examiner.